# EUROPEAN PATENT SPECIFICATION

(11) **EP 0 024 506 B1**
(45) Date of publication and mention of the grant of the patent: **12.09.1984**
(21) Application number: 80103687.2
(22) Date of filing: 30.06.1980
(51) Int. Cl.: B22D 11/04, B22D 11/06

(54) **Apparatus and method for chill casting of metal strip employing a chromium chill surface**
Apparat und Verfahren für das Kokillengiessen eines Metallbandes unter Verwendung einer Kokille mit chrombeschichteter Oberfläche
Dispositif et procédé pour la coulée en lingotière de bandes métalliques, en employant une lingotière à surface chromée

(30) Priority: 13.08.1979 US 66254
(43) Date of publication of application: 11.03.1981
(73) Proprietor: ALLIED CORPORATION, Morristown New Jersey 07960 (US)
(72) Inventor: Freilich, Alfred, Livingston, New Jersey 07039 (US)
(74) Representative: Weber, Dieter, Dr.

## Description

### Background of the Invention and the Prior Art

Methods are known for making continuous metal strip, of crystalline as well as amorphous (glassy) structure, directly from the melt by depositing molten metal onto the surface of a rapidly moving chill body whereon it is quenched to the solid state.

The US-A-4 142 571 describes an apparatus for making thin metal sections directly from the melt by depositing molten metal onto the surface of a rapidly moving chill body comprising a chill body constructed of a metal selected from the group consisting of copper, silver, molybdenum and alloys thereof, having a surface coating of chromium and having a sur_{'}- face adapted to receive molten metal to be deposited thereon for rapid quenching together with means functionally connected with said chill body for depositing molten metal onto its surface. Metal strips prepared by means of such an apparatus having a highly polished chill surface as recommended in column 8, line 4 of the US-A-4 142 571 tend to have non-uniform properties and bad ductility.

The surface of the chill body must meet several requirements. First, it must be wetted by the molten metal, or else formation of continuous strip will not take place. Second, it must be non-reactive with the molten metal, that is to say the molten metal must not attack, and must not weld to the chill surface, or else the strip cannot be cleanly separated therefrom. Third, it must have good thermal conductivity to permit rapid removal of heat as is necessary to effect rapid solidification of the molten metal to permit formation of the molten metal, to permit formation of the glassy structure, and to optimize the properties of the metallic glass strip, especially to optimize its magnetic properties. Lastly, it must have sufficient wear resistance in continuous production of metal strip by the above-described quench casting process. Wear resistance is an extremely important aspect of chill body performance. High heat conductivity metals previously proposed to serve as chill body surface, such as copper, beryllium copper or silver, do not have the desired wear characteristics. Others, such as stainless steel, which would be expected to have good wear characteristics, fall short in other respects, such as failure to provide sufficient wetting, or good thermal conductivity.

The objective of the invention was to improve the known method and apparatus for making metal strip directly from the melt to obtain metal strips having properties as uniform as possible and having a good ductility.

The inventive method for making metal strip directly from the melt by depositing the molten metal onto the surface of a rapidly moving chill body having a heat-extracting metal selected from the group consisting of copper, silver, molybdenum and alloys thereof and having a surface coating of chromium, is characterized in that the coating of chromium has a thickness of from 0.002 to 0.15 mm and a surface roughness of from 0.25 to 3.0 µm.

The invention provides also an improvement of the apparatus for making thin metal sections directly from the melt by depositing molten metal onto the surface of a rapidly moving chill body comprising a chill body constructed of a metal selected from the group consisting of copper, silver, molybdenum and alloys thereof, having a surface coating of chromium and having a surface adapted to receive molten metal to be deposited thereon for rapid quenching together with means functionally connected with said chill body for deporting molten metal onto its surface, which is c ac- terized in that the coating of chromium a thickness from 0.002 to 0.15mm and .r-face roughness of 0.25 to 3 ,um.

By the chill body being constructed of copper, silver, molybdenum or alloys thereof it is meant that these metals fumish the heat extracting member of the chill body, or the "heat sink", which absorbs the heat of the molten metal to effect rapid quenching thereof to the solid state, desirably at rates in the order of 10⁴⁻10^{B} °K/sec, or higher, as may be required for formation of metallic glass bodies from glass-forming alloy melts. This therefore does not mean that in the constructing of the chill body other metals may not be employed, e.g. for structural purposes, such as reinforcement, and chill bodies incorporating other metals are intended to be within their scope of the appended claims.

It was surprisingly found that the above-described chromium surface coat, of the specified thickness and critically defined surface texture (surface roughness) is readily wetted by the molten metal, especially by iron, nickel and/or cobalt-based alloys which upon rapid quenching from the melt form amorphous structures (metallic glasses). Particularly good wetting seems to be obtained with glass-forming, iron-based, boron-containing metal melts wherein the metal component predominantly comprises iron. There are of considerable practical interest because of their outstanding soft magnetic properties, which make them eminently suitable for use in electromagnetic induction devices. The particular chromium surface further provides for good adhesion of the solidified metal strip, which is essential to effect thorough quenching of the metal if a ductile, amorphous metal strip is desired, yet is also affords clean release of the solidified strip from the surface. It is believed that the surprising improvement in soft magnetic properties of iron-based, boron-containing metallic glasses quenched on the chill body of the present invention, which has been observed, is due to such good adhesion and thorough quenching.

Lastly, the particular chromium-coated chill bodies of the present invention combine the above-described advantageous wetting and quenching properties with excellent wear resistance.

The benefits of the above-described chill bodies having a chromium surface of specific thickness and surface structure in the process of making metal strip directly from the metal by depositing the molten metal onto the rapidly moving surface of a chill body are obtained regardless of the configuration of the chill body. That is to say, the chill body may be a rapidly rotating drum of which the exterior surface is used as the chill surface; it may be a rapidly rotating cylinder whereof the inner surface furnishes the chill surface, a moving belt, a cup- shaped structure, or any other structure. Further, any means of depositing the molten metal onto the chill surface, e.g. jetting, flowing, dragging, dipping and others may be employed, without restriction.

For purposes of the present invention, a strip is a slender body whose transverse dimensions are much less than its length. In that context, strips may be bodies such as ribbons, sheets or wires, of regular or irregular cross-section.

### Brief Description of the Drawings

The annexed drawings further illustrate the present invention.
Fig. 1 is a cross-sectional view of an annular chill roll, the exterior surface of which is coated with a chromium in accordance with the present invention;
Fig. 2 is a cross-sectional view of an annular chill roll having a ring of chromium-coated molybdenum inserted in its surface;
Fig. 3 is a cross-sectional view of a cylindrical chill body having an inner chromium-coated chill surface inclined with respect to the axis of rotation;
Fig. 4 is a side view in partial cross-section showing means for jetting molten metal onto a rotating chill roll, and a rotating chill roll- provided with a chromium-coated chill surface;
Fig. 5 is a somewhat simplified perspective view of apparatus including means for depositing molten metal onto a chill surface in the form of a moving endless belt having a chromium surface.

### Detailed Description of the Invention, of the Preferred Embodiments, and of the Best Mode Presently Contemplated For its Practice

It has now been found that for use in such chill casting processes, chill bodies having heat extracting members of silver, copper, molybdenum or alloys thereof, which heat extracting members have a chromium-coated chill surface of the construction according to the invention, have very desirable properties, especially for casting metallic glass strips of iron-based boron-containing alloys.

The chromium coating must be at least about 0.002 millimeter thick or else it is of little or no benefit, inter alia for the reason that it provides insufficient wear resistance. On the other hand, it may not be thicker than about 0.15 millimeters. It was found that substantially thicker chromium coatings result in insufficient quenching of the melt, and in general deterioration in physical properties of glassy metal strip cast thereon, especially loss in ductility and of magnetic properties, e.g. reduced maximum induction and permeability. Good results are obtained with chromium coatings having thickness of from about 0.01 to about 0.1 millimeter, more preferably of from about 0.01 to about 0.075 millimeter.

The second critical element is the surface texture of the chromium coat. It has been thought by those skilled in the metallic glass casting art that it would be difficult or impossible to cast metallic glass strip by quench casting techniques on chromium surfaces, principally because of their relatively low heat conductivity. Not only that, it was further found that such strip, when cast on a smooth chromium surface, even a smooth, thin chromium surface of thickness within the range of that contemplated by the present invention, fails to adequately wet the surface and to adhere to the surface sufficiently to obtain good quenching of the strip. Consequently, strip cast on smooth chromium surfaces tends to be brittle, to have non-uniform properties, and to lack good magnetic properties. Such strip is commercially unacceptable.

Insufficient surface roughness below about 0.25 micrometers will tend to result in the above-described shortcomings of a smooth chromium surface. A higher degree of surface roughness above about 3.0 micrometers, while generally providing sufficient quench rate and adhesion, results in strip having undesirably high roughness on the surface cast in contact with the chill surface. Good results are obtained with chill surface texture corresponding to surface roughness of from 0.5 to about 2.0 micrometers, preferably of from about 0.6 to about 1.5 micrometers. The most preferred surface texture is a "satin finish", within the above- stated ranges of surface roughness, a satin finish being defined as a surface texture without visibly discernible lay, that is to say that surface roughness is the same measured in any direction. However, a satin finish, while providing the best results, is not absolutely necessary, and acceptable results are also obtained under conditions of discernible lay, such as where the finish runs longitudinal or transverse of the casting direction, or in any direction therebetween.

When amorphous metal strips are made by jetting molten glass forming alloy against the surface of a rapidly rotating chill body as, e.g., described in US-A-4,077,462 or in US-A-3,856,074 the surface of the chill body becomes gradually eroded. A rough, uneven track is developed around the periphery of the chill body surface whereon casting of the strip takes place. Further casting into the same track produces strip of unacceptable quality, having a rough surface and ragged edges. The problem of chill surface wear in these processes is even more acute when casting takes place under vacuum. The absence of an intervening gas layer in vacuum casting allows a larger area of the chill surface to be impacted and wetted by the molten jet. Another factor which leads to severe wear on conventional chill surfaces is inclusion in the alloy being cast of appreciable amounts of refractory metals, e.g., molybdenum, tungsten, chromium, hafnium, iridium, niobium, osmium, platinum, rhenium, rhodium, ruthenium, tantalum, thorium, vanadium, and zirconium. Hence, use of the chill surface of the present invention is particularly advantageous when casting under vacuum (say under absolute pressure of less than about 2 mm Hg), or when casting glass-forming alloys containing one or more refractory metals, and especially when casting such alloys under vacuum.

The form of the chill body and the mode of the casting operation are not critical for purposes of the present invention. For example casting may take place against the peripheral surface of a rapidly rotating drum by jetting molten metal against that surface, as disclosed in the above-mentioned US-A-4,077,462 and 3,856,074. Casting may take place against the exterior surface of a rotating drum by drawing out the metal from a meniscus formed at a slotted nozzle, as described in US-A-3,522,836 or from a pendant, unconfined drop of molten metal as described in US-A-3,896,203. Alternatively, the peripheral surface of the rotating chill drum may be dipped into a bath of molten metal as described in US-A-3,861,450, or the molten metal may be deposited under pressure from a slotted nozzle onto the chill surface, as described in US-A-4.,142,571. Furthermore, the chill surface may be furnished by the interior surface of a rotating cylinder, as described in US-A-3,881,540 and US-A-3,881,542 or as shown in Trans. Met. Soc. AIME, 245 (1969), pages 2475-6. Also, casting may take place into the nip of two counter-rotating chill rolls, as for example described in US-A-3,881,541 and in Rev. Sci. Instrum. 41, 1237 (1970). Moreover, the chill surface may be furnished by the open concave surface of a rapidly rotating cup as disclosed in US-A-2,825,108; or a moving belt, desirably a moving endless belt, as described in US-A-2,886,866. The advantages of the use of the specific chromium-coated chill body of the present invention are obtained regardless of the construction of the chill body, and regardless of the means for depositing the molten metal onto the chill surface, that is to say whether by jetting, dragging from a meniscus or a pendant drop, forcing it through a slotted nozzle located in close proximity to the chill surface or by dipping into a bath of molten metal, or by any other suitable means.

The chromium coating or plating is suitably applied to the substrate of copper, silver, molybdenum or alloys thereof by means of electroplating, using conventional electroplating procedures, although other the procedures may be employed, if desired. Methods of chromium plating are well known, and generally involve passing a d.c. current through a suitable plating bath, e.g. one containing chromic acid together with a suitable "catalyst", typically sulfate ion provided by sulfuric acid, and using the surface to be plated as the cathode. The chromium plating operation can be facilitated, and the adhesion of the chromium coating can be improved by first applying to the surface to be plated a thin (e.g. less than about 0.01 millimeter thick) "strike" coat of nickel, as is conventional in chromium plating operation.

The surface texture, i.e. the above-described surface roughness, may be provided by treating the chill surface by suitable means before or after the chromium plating operation, or both before and after the chromium plating operation, with suitable abrasive. For ease of treatment, and to protect the integrity of the chromium coat, surface treatment before the chromium plating operation is preferred. Surface texture can suitably be obtained by abrading the chill surface with a suitable abrasive, such as emery cloth and the like, or by impinging a suitable finely divided hard powder against the chill surface, or by similar means. A very effective means involves "slurry honing", which involves impinging a fluid stream containing finely divided suspended abrasive particles against the surface to be roughened.

In any event, methods of plating and of providing the specific surface texture are well known and are not part of the present invention.

When the chill body is to be made of molybdenum, it can be made by procedures usually employed for fabrication of molybdenum, including machining from solid stock, such as cast pieces, or fabrication by known powder metallurgical methods. A particularly desirable embodiment of the present invention is a composite chill body, especially a chill roll, made of copper provided with a hoop of molybdenum, as illustrated in Figs. 1 and 2. The casting surface provided by the molybdenum is chromium plated and has the above-described surface texture. With reference to Fig. 1, chill roll 1 made of copper is mounted for rotation on shaft 2. The exterior surface of chill roll 1 is provided with a hoop of molybdenum 3. In Fig. 1, the hoop of molybdenum covers the total peripheral surface of the chill roll. The molybdenum hoop may be affixed to the copper chill roll, e.g. by shrink fitting. Alternatively, a molybdenum surface may be provided by any other conventional surface coating method, as for example oxyacetylene spraying, a method which involves feeding a molybdenum wire into the cone of an oxygen/acetylene flame to melt the metal, and then propelling the molten metal in droplet form against the surface to be coated. Other suitable methods include plasma arc spraying and conventional cladding procedures.

Another embodiment of the present invention utilizing a copper-beryllium chill body from the conventional copper-beryllium alloys is also suitable.

Detailed design and construction of apparatus of the present invention is within the capability of any competent worker skilled in the art.

The following Example further illustrates the present invention and sets forth the best mode presently contemplated for its practice.

### Example and Comparative Test

Apparatus employed was similar to that depicted in Fig. 4 employing a water-cooled copper chill roll having a 0.025 millimeter thick satin finish chromium coating with surface roughness of about 0.76-0.80 micrometers. The chill roll had a diameter of 38.1 cm, and it was rotated at a speed to provide peripheral velocity of from 914 to 1067 meter/min. The nozzle for depositing the molten metal had an orifice of 2.54 cm length and 0.5 mm width. The gap between the chill surface and the nozzle was about 0.25 mm.

Alloy of composition Fe₈₁B_{13.5}Si_{3.5}C₂ (atom percent) was ejected through the nozzle into contact with the rotating chill surface under pressure at the rate of about 4.53 kg/min. It solidified on the surface of the chill roll into a strip 2.54 cm wide and about 0.038 cm thick.

A comparative run employing a copper chill roll without the above-described chromium coating, but under otherwise identical conditions, was made. Properties of the strip obtained in the Example and in the comparative run are summarized in the Table, below.

It was noted that the chromium coated chill roll did not show any discernible wear after 110 kg of metal had been cast in 12 consecutive runs of about equal size, each on the same "track". A plain copper wheel would show considerable wear after a single run, and the chill surface would require "dressing" after each individual run to restore the chill surface to the necessary degree of smoothness required to make strip of acceptable surface characteristics.

As the data in the Table demonstrate, the strip cast on the chromium plated surface having specific surface texture has substantially improved magnetic properties as compared to strip cast in conventional manner on a copper chill surface. Differences in magnetic properties from beginning to the end of the run are substantially less in each instance. Transformers made from strip cast on such chromium plated chill roll will have substantially improved efficiency, in that they will have greatly reduced core losses, and greatly reduced VA demand.

Since various changes and modifications may be made in the invention without departing from the scope and essential characteristics thereof, it is intended that all matter contained in the above description shall be interpreted as illustrative only, the invention being limited only by the scope of the appended claims.

## Claims

1. Method for making metal strip directly from the melt by depositing the molten metal onto the surface of a rapidly moving chill body having a heat-extracting metal selected from the group consisting of copper, silver, molybdenum and alloys thereof and having a surface coating of chromium, characterized in that, the coating of chromium has a thickness of from 0.002 to 0.15 mm and a surface roughness of from 0.25 to 3.µ µm.

2. The method of claim 1 wherein the chill body is a chill roll and the molten metal is deposited into its peripheral surface and wherein the metal is one which, upon rapid quenching from the melt, forms an amorphous (glassy) body.

3. The method of claim 1 wherein the chill body is an endless belt constructed of copper-beryllium alloy.

4. Apparatus for making thin metal sections directly from the melt by depositing molten metal onto the surface of a rapidly moving chill body comprising a chill body constructed of a metal selected from the group consisting of copper, silver, molybdenum and alloys thereof, having a surface coating of chromium and having a surface adapted to receive molten metal to be deposited thereon for rapid quenching together with means functionally connected with said chill body for depositing molten metal onto its surface, characterized in that the coating of chromium has a thickness of from 0.002 to 0.15 mm and a surface roughness of 0.25 to 3,am.

5. The apparatus of claim 4 wherein the surface coating has a satin finish without discernible lay.

6. The apparatus of claim 5 wherein the chill body is a chill roll.

7. The apparatus of claim 6 wherein the chill roll is constructed of copper-beryllium alloy.

8. The apparatus of claim 6 wherein the chill roll is constructed of molybdenum.

9. The apparatus of claim 4 wherein the chill body is an endless belt.

10. The apparatus of claim 9 wherein the endless belt is constructed of copper-beryllium alloy.

## Revendications

1. Procédé de fabrication d'une bande de métal directement à partir du métal en fusion par dépôt de ce dernier sur la surface d'un corps de refroidissement et trempe, se déplaçant rapidement, et constitué par un métal absorbant la chaleur sélectionné dans le groupe comprenant le cuivre, l'argent, l'molybdène et des alliages de ces derniers, et présentant un revêtement de surface en chrome caractérisé en ce que le revêtement de chrome a une épaisseur comprise entre 0,002 et 0,15 mm, et une irrégularité de surface de 0,25 à 3,µ µm.

2. Procédé selon la revendication 1 dans lequel le corps de refroidissement est un rouleau et le métal fondu est déposé sur sa surface périphérique, et dans lequel le métal est tel que, lors de la trempe rapide à partir de l'état fondu, il constitue un corps amorphe (vitreux).

3. Procédé selon la revendication 1 dans lequel le corps de refroidissement est une courroie sans fin réalisée en alliage cuivre-béryllium.

4. Appareil pour fabriquer des sections de métal de faible épaisseur directement à partir du métal en fusion par dépôt de ce dernier à la surface d'un corps de refroidissement et trempe se déplaçant rapidement et comprenant un corps réalisé en un métal choisi dans le groupe comportant le cuivre, l'argent, le molybdène et des alliages de ces derniers, ledit corps ayant un revêtement de surface en chrome et présentant une surface susceptible de recevoir le métal en fusion qu'il y a lieu d'y déposer en vue de sa trempe rapide ainsi que des moyens reliés fonctionnellement audit corps pour déposer le métal en fusion sur sa surface caractérisé en ce que le revêtement de chrome a une épaisseur comprise entre 0,002 et 0,15 mm et présente une irrégularité de surface de 0,25 à 3 um.

5. Appareil selon la revendication 4 dans lequel le revêtement de surface a un fini satiné et ne présente pas de rayures perceptibles.

6. Appareil selon la revendication 5 dans lequel le corps de refroidissement est un rouleau.

7. Appareil selon la revendication 6 dans lequel le rouleau est réalisé en alliage de cuivre- béryllium.

8. Appareil selon la revendication 6 dans lequel le rouleau est réalisé en molybdène.

9. Appareil selon la revendication 4 dans lequel le corps de refroidissement est une courroie sans fin.

10. Appareil selon la revendication 9 dans lequel la courroie sans fin est réalisée en alliage de cuivre-molybdène.

## Patentansprüche

1. Verfahren zur Herstellung eines Metallstreifens direkt aus der Schmelze durch Ablagerung des geschmolzenen Metalles auf der Oberfläche eines sich schnell bewegenden Kühlkörpers mit einem Wärme entziehenden Metall aus der Gruppe Kupfer, Silber, Molybdän und den Legierungen derselben und mit einem Oberflächenüberzug aus Chrom, dadurch gekennzeichnet, daß der Chromüberzug eine Dicke von 0,002 bis 0,15 mm und eine Oberflächenrauhheit von 0,25 bis 3,O,um hat.

2. Verfahren nach Anspruch 1, bei dem der Kühlkörper eine Kühlwalze ist und das geschmolzene Metall in ihrer Umfangsfläche abgelagert wird und das Metall ein solches ist, das beim raschen Abschrecken aus der Schmelze einen amorphen (glasartigen) Körper bildet.

3. Verfahren nach Anspruch 1, bei dem der Kühlkörper ein Endlosband aus einer Kupfer-Beryllium-Legierung ist.

4. Vorrichtung zur Herstellung dünner Metallabschnitte direkt aus der Schmelze durch Ablagerung von geschmolzenem Metall auf der Oberfläche eines sich schnell bewegenden Kühlkörpers mit einem Kühlkörper, der aus einem Metall aus der Gruppe Kupfer, Silber, Molybdän und den Legierungen derselben besteht, einen Oberflächenüberzug aus Chrom hat und eine Oberfläche besitzt, die so ausgebildet ist, daß sie hierauf abzulagerndes geschmolzenes Metall für ein rasches Abschrecken aufnimmt, zusammen mit funktionell mit dem Kühlkörper verbundenen Einrichtungen zur Ablagerung von geschmolzenem Metall auf seiner Oberfläche, dadurch gekennzeichnet, daß der Chromüberzug eine Dicke von 0,002 bis 0,15 mm und eine Oberflächenrauhheit von 0,25 bis 3 _{M}m hat.

5. Vorrichtung nach Anspruch 4, bei der der Oberflächenüberzug ohne wahrnehmbare Strichrichtung mattiert ist.

6. Vorrichtung nach Anspruch 5, bei der der Kühlkörper eine Kühlwalze ist.

7. Vorrichtung nach Anspruch 6, bei der die Kühlwalze aus Kupfer-Beryllium-Legierung besteht.

8. Vorrichtung nach Anspruch 6, bei der die Kühlwalze aus Molybdän besteht.

9. Vorrichtung nach Anspruch 4, bei der die Kühlwalze ein Endlosband ist.

10. Vorrichtung nach Anspruch 9, bei der das Endlosband aus Kupfer-Beryllium-Legierung besteht.
